

Aug. 5, 1930.

V. ENGELHARDT ET AL

1,772,074

## METHOD OF PRODUCING GALVANIC COATINGS

Filed Feb. 9, 1926



Fig. 2

Inventors:  
Victor Engelhardt  
and Kurt Mlig  
by Lorka, Kellenbeck & Farley  
Attorneys.

## UNITED STATES PATENT OFFICE

VICTOR ENGELHARDT, OF BERLIN-CHARLOTTENBERG, AND KURT ILLIG, OF BERLIN-WILMERSDORF, GERMANY, ASSIGNEES TO SIEMENS & HALSKE, AKTIENGESELLSCHAFT, OF SIEMENSSTADT, NEAR BERLIN, GERMANY, A CORPORATION OF GERMANY

## METHOD OF PRODUCING GALVANIC COATINGS

Application filed February 9, 1926, Serial No. 87,020, and in Germany October 17, 1925.

The present invention relates to the production of galvanic coatings on bodies, especially on narrow tubes. In obtaining durable coatings it is often necessary—for example when producing a chromium coating—to work with an electrolyte which attacks nearly all substances, especially metals in the unpolarized condition, giving rise to impurities in the electrolyte. In such case it is therefore necessary to use the hollow body as the cathode and, furthermore, when making internal coatings, to use it as electrolyzer. Again, in the case of the production of coatings on comparatively narrow tubes, there is present in the internal hollow space of the tube only a small quantity of the electrolyte which, on the passage of the electric current, is liable to become heated to boiling point by the Joule's heat developed. The whirling of the liquid resulting in this case and the rising gas bubbles then make the production of a satisfactory inner coating for the tube impossible.

The invention relates to a process for obviating the disadvantages mentioned and to an apparatus that is especially advantageous for the carrying out of this process, particularly for producing chromium coatings, but is also applicable to other electroplating processes in which difficulties similar to those set forth above are experienced.

In carrying out the new method for producing galvanic coatings on bodies, the body to be coated is used as the cathode and brought into an electrolyzer. According to the invention an anode arrangement continuously dipping into the electrolyte is moved with relation to the cathode body along those parts of the surface which are to be coated. The velocity of this movement is so chosen that the resulting coating is of the desired thickness at every point. It is immaterial to the invention whether only the body or only the anode arrangement or both parts be moved as long as there is a relative motion. The essential advantage of the new method with regard to other well-known methods consists in the fact that the new method may be employed for producing outer

or inner galvanic coatings on bodies of any form, and especially on narrow tubes.

In the drawings there is shown an example of an apparatus for carrying out the new process. Figure 1 is a longitudinal section through the apparatus and Figure 2 is a section on the line AB of Figure 1.

In an electrolyzer or electrolytic vessel 1 that contains the electrolyte 2 a hollow body 3 is arranged so as to be fixed in position, for example by being suspended by means of a wire 18, and is connected in such a manner that it will become the cathode. For instance, the suspension wire 18 may be employed as a conductor connected to the negative wire 60 of a direct current line 14, 15. The anode is constituted by the bodies 4 and 5 which are movably arranged, by means of suspension wires 9 and 10 passing over rollers 6, 7 and 8, in the interior and on the exterior respectively of the hollow body 3. The anode 4 is shown as a continuous unitary solid body, but may if desired also be in the form of a hollow body—for example, a hollow cylinder. The wires 9 and 10 can likewise serve 75 as current conductors by connecting them to the positive wire of the line 14, 15. On the anodes 4 and 5, the length of which is preferably about one-tenth of that of the hollow body, there are arranged projections 11 and 12 of insulating material for the purpose of obviating short-circuiting between the electrodes. Instead of the lug-like projections shown, centering beads of insulating material may be provided on the anodes. These 80 insulators also serve the purpose of guiding the anodes with relation to the cathodes and have the effect of maintaining a nearly constant spacing between the anodes and cathode, and consequently of maintaining a nearly 85 constant current density at the cathode, this being of great importance in plating with chromium from chromic acid solutions. A cock 13 arranged on the vessel 1 serves for the introduction of fresh electrolyte. The 90 apparatus is preferably employed in the following manner:

First, the anodes 4 and 5 are let down until their lower edges are approximately on a level with that of the hollow body 3. The level of 100

the electrolyte is then preferably so chosen that it is only at a small distance above the upper edges of the anodes. Thereupon, the current is switched on by means of the switch 5 17 and the anodes 4 and 5 are gradually raised by means of the wires 9 and 10 by a handle 16, connected to the wires 9, 10. Instead of the handle 16 any suitable automatically working machine—for example a clock-work—may be used for the same purpose. The cock 13 is at the same time opened to such an extent that the level of the electrolyte is always maintained a little—for example, a few centimetres—above the upper edges of 10 the anodes 4 and 5. The movement of the anodes preferably takes place at a uniform velocity which is so chosen that the coating produced is of the desired thickness.

The insulating centering pieces, which may 20 also be secured to the upper and the lower ends of the anodes 4 and 5 (for instance in the form of tooth-like discs), prevent the anodes 4 and 5 as they move vertically in a straight path, from striking against the 25 cathode 3.

In this way, the whole hollow body becomes gradually coated. It is self-evident that if a galvanic coating is to be produced only on the interior or only on the exterior surface 30 of a body, the particular anode which at the time being is not to be used, is removed from the bath.

In the new process a slight dispersion upwardly and downwardly from the edges of 35 the anode generally takes place which results even before the actual galvanization, in the production of a coating similar to that produced by breathing on a surface on the parts of the body that are encountered by the dispersed substance. The advantage of this is 40 that the body is not attacked by the electrolyte and, in addition, the main coating produced on direct juxtaposition of anode and cathode adheres with extraordinary firmness.

It will be noted that both the inner and the outer surfaces of the hollow body 3 are in contact with the electrolyte, and that the liquid in the two annular zones through which the current passes from the anodes 4 and 5 45 to the cathode formed by the body 3, is in communication with a much larger body of liquid. In the deposition of chromium and of some other metals, considerable heat is developed. This heat, which is liable to interfere with the success of the plating operation, is readily absorbed by, and dissipated in, the large body of electrolyte in which the body 3 and both anodes 4, 5 are immersed.

The new process is therefore especially advantageous in the case of the production of chromium coatings; it can, however, be employed for the production of any other desired coatings, especially in the case of oxidizing electrolytes and hollow bodies of 50 easily attackable metal.

What we claim as our invention and desire to secure by Letters Patent is:

1. The method of producing a galvanic chromium coating on a hollow body, which consists in dipping the hollow body into an electrolyte suitable for chromium deposition, in such a manner that said electrolyte will be in contact with the inner surface and with the lower end of the said hollow body, placing within said body an anode which is a small fraction of the length of said hollow body, passing an electric current from said anode through the electrolyte to said body, the latter serving as a cathode, and effecting relative movement of anode and cathode lengthwise of said hollow body, the anode, at the beginning of such movement, being adjacent to the lower end of said body, and adding quantities of the electrolyte to keep the level of the electrolyte a small distance above the upper edge of said anode. 55

2. The method of producing a galvanic chromium coating on a hollow body, which consists in dipping the hollow body into an electrolyte suitable for chromium deposition, in such a manner that said electrolyte will be in contact with the inner surface and with the lower end of the said hollow body, placing within said body an anode which is a small fraction of the length of said hollow body, passing an electric current from said anode through the electrolyte to said body, the latter serving as a cathode, effecting relative movement of anode and cathode lengthwise of said body, in a vertical direction, and adding such quantities of electrolyte that the level of the electrolyte will be kept a small distance above the upper edge of the said anode. 95

3. The method of producing a galvanic chromium coating on a hollow body, which consists in dipping the hollow body into an electrolyte suitable for chromium deposition, in such a manner that said electrolyte will be in contact with the outer surface and with the lower end of the said hollow body as well as with the inner surface thereof, placing an anode exteriorly of said body and an anode within such body, each of said anodes being a small fraction of the length of said hollow body, passing an electric current through said electrolyte from said anodes to said body, the latter serving as a cathode, and moving said anodes lengthwise of said hollow body from the bottom thereof to the top, and adding quantities of the electrolyte to keep the level of the electrolyte a small distance above the upper edges of said anodes. 115

4. Apparatus for producing an inner galvanic chromium coating on a tubular body, comprising in combination a vessel adapted to contain an electrolyte suitable for chromium deposition and the tubular body to be coated, a wire for connecting the said tubu- 125

- lar body with the negative pole of a source of electric current, means for suspending the said tubular body stationary in the said vessel at a distance above the bottom of the said vessel, an anode suspended within said body, said anode being a small fraction of the length of said hollow body, insulating means to guide and to keep said anode out of contact with said tubular body, and means for longitudinally moving the said anode along the inner surface of the said tubular body.
5. Apparatus for producing an inner galvanic chromium coating on a tubular body, comprising in combination a vessel adapted to contain an electrolyte suitable for chromium deposition and the tubular body to be coated, a wire for connecting the said tubular body with the negative pole of a source of electric current, means for suspending the said tubular body stationary in the said vessel at a distance above the bottom of the said vessel, an anode suspended within said body, said anode being a small fraction of the length of said hollow body, insulating means to guide and to keep said anode out of contact with said tubular body, means for moving the said anode along the inner surface of the said tubular body from the bottom to the top, and a device for introducing such quantities of electrolyte into the said vessel that the level of the electrolyte in the said vessel both within and without the said tubular body will be kept a small distance above the upper end of the said anode.
20. Apparatus for producing a chromium coating on both the outer and the inner surfaces of a tube, comprising in combination, a vessel adapted to contain an electrolyte suitable for chromium deposition and the tube to be coated, means for suspending the said tube in a vertical position in the said vessel and for connecting the said tube with the negative pole of a source of electric current, an anode suspended within the said tube, insulating means for guiding and for keeping said anode out of contact with said tube, a wire connected to said anode, an annular anode exteriorly of the said tube, each of said anodes being a small fraction of the length of said hollow body, insulating means for guiding and for keeping said second anode out of contact with said tube, another wire connected to said second anode, and means adapted to move the said anodes longitudinally along the inner and the outer surfaces of the tube respectively.
25. The method of electroplating a conducting hollow body on both its outer and its inner surfaces, which consists in dipping it into an electrolyte in such a manner that both of said surfaces of the body will be in contact with the electrolyte, placing two anodes each of relatively small length compared with that of said body adjacent to said body, one interiorly and the other exteriorly thereof, effect-
- ing relative movement between said anodes and said body, and passing an electric current through the electrolyte from said anodes to said body, the latter serving as a cathode.
8. Apparatus for electroplating conducting hollow bodies both on their inner and on their outer surfaces, comprising a vessel adapted to contain an electrolyte and the body to be plated, two spaced anodes so located that the article to be coated may be placed between them, said anodes each being of a length which is relatively small as compared with the height of said vessel, connections for causing an electric current to pass through the electrolyte from said anodes to said body, and means for effecting relative longitudinal movement between said anodes and said body.
15. Apparatus for electroplating conducting hollow bodies both on their inner and on their outer surfaces, comprising a vessel adapted to contain an electrolyte and the body to be plated, two spaced anodes so located that the article to be coated may be placed between them, said anodes each being of a length which is relatively small as compared with the height of said vessel, connections for causing an electric current to pass through the electrolyte from said anodes to said body, and insulating means carried by each anode and projecting therefrom toward the other anode to prevent contact of said body with either anode, and to guide the latter.
20. In testimony whereof we affix our signatures.
100. VICTOR ENGELHARDT.  
KURT ILLIG.
- 105.
- 110.
- 115.
- 120.
- 125.
- 130.